

# UNITED STATES PATENT OFFICE.

CHARLES E. HITE, OF BURLINGTON, NEW JERSEY.

## PROCESS OF BRIQUETING COAL.

941,454.

Specification of Letters Patent. Patented Nov. 30, 1909.

No Drawing

Application filed March 28, 1909. Serial No. 485,901.

To all whom it may concern:

Be it known that I, CHARLES E. HITE, a citizen of the United States, residing at Burlington, in the county of Burlington and State of New Jersey, have invented a new and useful Process of Briqueting Coal, of which the following is a specification.

My invention relates to an improved process of forming a binder for the briqueting of fine coal.

The object of my invention is the production of a binder, for binding or cementing under pressure, fine particles of coal into a compact body.

The commercial conditions attending the manufacture of a good briqueted coal, are such that it is necessary to produce a binder as cheaply as possible, and that the binder should be composed of materials easily obtained at various localities throughout the country. The binder should be made of materials which will add to, or at least, not detract from, the coal's heat value. The materials used in the binder should be of such a nature that they will not add materially to the percentage of ash formed after combustion. These conditions led me to investigate oils, some of which absorb oxygen readily on exposure to the atmosphere, also the fatty acids, and crude petroleum. The problem was how to distribute a minimum amount of an oil, a fatty acid or crude petroleum over a given quantity of fine or pulverized coal. This I have successfully accomplished by making an emulsion, using a flour paste as the emulsifying medium or emulsifier for the oil, fatty acids or petroleum. When the emulsion is formed, the flour which contains glutinous or amyloseous matter, having been mixed with water and subjected to heat until thoroughly cooked, which is indicated by the bursting of the starch granules, and to which has been added the oil, fatty acid or petroleum, forms a simple, efficient, inexpensive medium for the distribution of the materials over a large area of fine coal. The fixed oils on exposure to the atmosphere, become oxidized, and with the glutinous and amyloseous substances in the paste form an excellent waterproof binder, when the same has been incorporated with the coal and briqueted. Just what change occurs with the fatty acids and crude petroleum, when emulsified and used for briqueting coal, has not been determined, but they become very hard when ex-

posed to the air, and seem to act in a measure like the fixed oils.

It is also the object of my invention to make a briquet which will stand a drop of 60 four or six feet without breaking, immediately after leaving the press, and which can be handled or shipped in a day or two after being made, with but small breakage occurring.

My object also is to make a briquet that will not disintegrate or crumble to pieces when completely immersed or submerged in water for several days, and which will get harder or firmer the longer it stands, 70 without being softened or disintegrated by the weather changes, moisture or rain.

These various objects I have attained in practice by means of an oil emulsion at a cost which is not prohibitory to the commercial success of my binder, and process.

The method or process together with the binder, is as follows: Slack, screenings, fine culm or coal pulverized by machinery, is first subjected to a heat of from 150° to 200° 80 centigrade for about fifteen minutes; (this does not mean however that the entire mass is brought to the temperature mentioned) the object of this being to drive off a certain percentage of the moisture present in the 85 coal, also to soften the particles of coal, causing them to compress closer together in the briquet machine than would otherwise occur were the coal not heated. It also allows the binder to enter the coal which previously contained moisture, thus preventing water from again entering the particles and causing the binder to lose its hold. After the coal has been so heated, there is run into it, a binder that has been previously prepared, which, as an example, consists of the following ingredients and proportions necessary for the briqueting of one ton of culm or pulverized coal. It is understood that the proportions may be changed to suit the 95 nature and kind of coal to be briqueted. Also the kind of oils, oily matter or oleaginous material used may be so varied in kind or quantity.

To 390 pounds of water are added 25 100 pounds of flour or other glutinous, or amyloseous substance and made into a paste of the proper consistency by cooking in a water jacketed kettle, stirring slowly. When the paste is nearly done, four or five pounds 1 of alum, aluminum sulfate, calcium chlorid, formaldehyde, or other preservative are add-

ed and thoroughly mixed in the paste. This prevents the paste from losing its efficiency. After this is done, about one gallon of linseed oil or other fixed oil is added to the 5 paste preferably while still hot, and stirred slowly; under these conditions the oil is thoroughly emulsified, forming an emulsion. Continue stirring slowly until cool and all steam has been freed from the paste. When 10 the emulsion is exposed to the air and sets or hardens, it will practically resist the action of water. After this emulsion has been added to the coal, the mass is thoroughly mixed in a mechanical mixer, and formed 15 into briquets by a suitable machine.

By means of an oil emulsion, a small quantity of oil is distributed over far more surface than could be accomplished in any other manner, and after the briquets have 20 stood for several days, the water having largely evaporated, and when a fixed oil is employed, the oil is oxidized, which together with the flour paste cements the particles of coal into a very dense hard mass, that has 25 enough elasticity to prevent the briquets from becoming too brittle or too easily broken.

As linseed oil is largely composed of the glycerids of isolinolenic, linolenic, linolie, 30 oleic, stearic, palmitic and myristic acids, in certain kinds of coal, oleic, stearic, palmic or other fatty acids may be substituted for the linseed or other fixed oil; the result being practically the same in forming an 35 emulsion, which could not be formed with water alone.

What I claim is:—

1. The process of making an emulsion binder, which consists in mixing with water 40 a glutinous or amylaceous substance such as flour, heating the same until the starch granules have burst, adding thereto a suitable quantity of oil and agitating the mixture, thereby forming an emulsion.
2. The process of making an emulsion 45 binder, which consists in mixing with water

a glutinous or amylaceous substance such as flour, heating the same until the starch granules have burst, adding thereto a suitable quantity of fixed oil such as linseed oil, 50 or fatty acids, or crude petroleum, stirring the mixture until an emulsion is formed, and adding thereto a suitable paste preservative.

3. The process of using flour paste as the 55 emulsifying medium, or emulsifier, for forming emulsions of oils, fatty acids or the crude petroleum.

4. The process of briquetting pulverized 60 or fine coal by mixing therewith a binder in the form of an oil emulsion, composed of flour paste and oil, fatty acids or crude petroleum, and subjecting the mixture to pressure.

5. The process of briquetting fine coal, 65 which consists in mixing the same with an oil emulsion binder, composed of flour paste and linseed oil or other fixed oil, to which is added calcium chlorid or other suitable preservative, and submitting the mixture to 70 pressure.

6. The process of briquetting fine coal by 75 mixing the same with a binder, composed of flour paste and ethereal salts, in the formation of which glycerin as the alcohol, and acids such as palmitic, stearic and oleic acids, take part, forming with the flour paste an oily emulsion, to which may be added a suitable preservative and submitting the same to pressure.

7. The process of briquetting pulverized 80 or fine coal, which consists in first heating the coal then mixing therewith a binder in the form of an oil emulsion, composed of flour paste, an oil, fatty acids, or crude 85 petroleum, to which has been added a suitable preservative, and subjecting the mixture to pressure.

CHARLES E. HITE.

Witnesses:

MAE HOFMANN,  
HOWARD S. OKIE.